

1

3,090,680

## GASOLINE COMPOSITION

Reid E. Sutton and John L. Bame, East Alton, Ill., assignors to Shell Oil Company, New York, N.Y., a corporation of Delaware  
No Drawing. Filed Mar. 29, 1960, Ser. No. 18,257  
6 Claims. (Cl. 44—69)

This invention relates to improved hydrocarbon fuel compositions and particularly to improved motor gasoline fuel compositions having high octane numbers.

Recent automotive design trends have been toward engines having greater power for the same size engine and more efficient utilization of the gasoline fuel. Engine designers have accomplished this largely by steadily raising the compression ratios of automotive engines, which has necessitated the use of fuels having increased resistance to detonation or spark knock. There is also an increased demand for aviation fuels having greater antiknock properties. It has heretofore been possible to manufacture such fuels from crude petroleum by the development and utilization of new hydrocarbon conversion and synthesis processes such as cracking, reforming, polymerization, and alkylation. The resistance to knock of the fuels from these processes is even further augmented by the addition of antiknock agents such as tetraethyllead (TEL), and, recently, methylcyclopentadienyl manganese tricarbonyl. Resistance to spark knock is, of course, evaluated as "octane number." Therefore, the demand for fuels having greater resistance to spark knock is manifested in the constantly increasing octane number of premium fuels. However, as the octane number of modern gasoline fuels has been raised, there has been a concomitant decrease in the susceptibility of such fuels to octane number improvement by addition of organometallic antiknock agents. It becomes less economical, therefore, to obtain greater resistance to spark knock by this means with higher octane number fuels. In addition, the amount of organo-metallic additive which is added to motor fuels may also be limited by consideration of the degree of toxicity imparted to the fuel containing such materials. For this reason, the maximum amount of tetraethyllead which may be added to commercial gasoline motor fuels is 3 or 4 cc./gal. (U.S.) and 6 cc./gal. (U.S.) for automotive and aviation fuels, respectively. Consequently, the degree of octane number improvement which can be obtained in this manner is limited. Organo-metallic antiknock additives are difficult to synthesize and are expensive. Their addition to fuels is thus limited to small concentrations by considerations of economics as well. Yet another limitation on the use of such antiknock additive-containing fuels is the tendency of the antiknock additives therein to lay down large quantities of deposits in the combustion chamber of the engine, which may contribute to an increase in the octane number of requirement of the engine. Because of these limiting factors on the use of conventional organo-metallic antiknock additives, the octane number obtainable from gasoline fuels made by conventional refining processes has also been limited.

There have been many attempts to solve this problem by the use of two or more antiknock agents. However, in most of these situations, the incremental increase in octane number obtained by adding the second antiknock agent has been considerably less than the octane number increase obtainable when the supplemental antiknock agent is added to the gasoline by itself. That is, the antiknock activity of the supplemental antiknock agent or of both antiknock agents is less, on the basis of the volume added, than either by itself. Consequently, even though significant increases in octane number are ob-

2

tainable, it has heretofore been uneconomical to obtain higher octane number motor gasoline in this manner.

It is therefore an object of this invention to provide improved gasoline fuel compositions. It is also an object of the invention to augment the efficacy of tetraethyllead as an antiknock additive in gasoline. It is a further object of the invention to provide higher antiknock quality in gasoline in an economical manner. It is still another object to provide hydrocarbon compositions which enhance the efficiency of antiknock additives added thereto. Another object is to attain the foregoing objects without detrimental side effects in the use of the fuel in gasoline engines. A still further object of the invention is to provide an improved antiknock additive concentrate composition.

The attainment of these and other objects will be apparent from the detailed description of the invention which is a gasoline motor fuel composition containing a tetraalkyllead compound as a primary antiknock agent and small but critical amounts of certain aromatic chromium tricarbonyls which by themselves exhibit no primary antiknock activity.

The use of organo-metallic compounds as primary antiknock agents has long been known, and countless numbers of these materials have been suggested, tried, and used with various degrees of success. The most widely used for many reasons, including availability, economy, and antiknock activity, are the tetraalkylleads, particularly tetraethyllead and tetramethyllead. However, it has now been found that certain aromatic chromium tricarbonyls, which possess essentially no primary antiknock activity when they are added to gasoline containing no other antiknock agent, nevertheless when added to leaded gasolines of selected composition as to hydrocarbon type and boiling range possess an extraordinary and unexpected co-antiknock activity. By co-antiknock activity, it is here meant that the secondary or co-antiknock agent causes the octane number of the gasoline containing both primary and secondary antiknock additives to be raised significantly above the level which is obtained by the primary antiknock agent alone, the co-antiknock effect being the result of co-action of the secondary with the primary additive rather than any primary antiknock properties of the secondary additive alone.

The addition of very small amounts of aromatic chromium tricarbonyls to fuels containing tetraalkyllead primary antiknock agents has been found to raise the octane number of the total mixture by as much as 5.0 octane numbers.

The aromatic chromium tricarbonyls which have been found to be effective co-antiknock agents with tetraalkyllead are represented by the empirical formula



wherein A is a monoaromatic compound corresponding to the following formula:



65 Within the context of the above formula, three of the R's are monovalent radicals selected from —H and —CH<sub>3</sub>, while one of them is a monovalent radical selected from —H, C<sub>n</sub>H<sub>2n+1</sub>, —OR,



wherein n is a whole number from 1 to 4 inclusively, and

the R's are —H, —CH<sub>3</sub> or together are tetramethylene (—CH<sub>2</sub>CH<sub>2</sub>CH<sub>2</sub>CH<sub>2</sub>—).

The foregoing class of aromatic chromium tricarbonyls, which are believed to be complexes, may be prepared by displacement of CO from Cr(CO)<sub>6</sub> by the aromatic. Examples of such aromatic chromium tricarbonyls which have been prepared and which may be used according to the invention are those according to the formula ACr(CO)<sub>3</sub> in which A is benzene, toluene, o-xylene, m-xylene, p-xylene, mesitylene, hexamethylbenzene, tetrahydronaphthalene (tetralin), methoxybenzene (anisole), methyl o-tolyl ether, methyl p-tolyl ether, aminobenzene (aniline), o-toluidine, m-toluidine, p-toluidine, N-methylaniline, NNdimethylaniline, NNdimethyltoluidine, methyl benzoate, benzyl alcohol, acetophenone, tert.-butylbenzene, phenyl acetate.

The extraordinary co-antiknock action of this unique class of complexes may best be seen by reference to the following example:

#### EXAMPLE I

A number of aromatic chromium tricarbonyls, each within the foregoing described class, were added to separate samples of a commercial gasoline blending component having a boiling range below about 400° F. and which had previously been leaded to a level of 3 cc. tetraethyllead (TEL) per U.S. gallon. The octane number of all the samples containing the co-antiknock or secondary additive and also a separate sample of each of the same gasoline blending components containing only 3 cc. TEL/gal. (U.S.) were determined by the Research Method (ASTM test designation D-357-53). To determine the increase in octane number obtained by adding small amounts of co-antiknock agent, the difference in the octane numbers of the samples with and without co-antiknock agent (Δ.O.N.) were calculated. The results are tabulated in the following Table I.

Table I

| Secondary antiknock agent                      | Concentration (millimoles/gal.) | Metal ratio (gms. Cr/gm. Pb) | Octane number enhancement (Δ O.N.) |
|------------------------------------------------|---------------------------------|------------------------------|------------------------------------|
| Mesitylene chromium tricarbonyl <sup>1</sup>   | 1                               | .016                         | 2.4                                |
|                                                | 2                               | .033                         | 3.0                                |
|                                                | 4                               | .065                         | 1.7                                |
|                                                | 8                               | .131                         | -0.7                               |
| Mesitylene chromium tricarbonyl <sup>2</sup>   | 1                               | .016                         | 5.0                                |
|                                                | 2                               | .033                         | 3.7                                |
| Toluene chromium tricarbonyl <sup>1</sup>      | 1                               | .016                         | 0.2                                |
|                                                | 2                               | .033                         | 1.2                                |
|                                                | 4                               | .065                         | 2.9                                |
|                                                | 8                               | .131                         | 3.6                                |
| Ortho xylene chromium tricarbonyl <sup>1</sup> | 1                               | .016                         | 2.0                                |
|                                                | 2                               | .033                         | 2.6                                |
|                                                | 8                               | .131                         | 0.0                                |

<sup>1</sup> In olefin-isobutane alkylate.

<sup>2</sup> In blend of naphthalenes: equal volumes of cyclohexane, cyclopentane, and methyl cyclopentane.

The data in the foregoing table show that large increases in octane number are obtainable at extremely low metal concentrations. In view of the fact that the increases obtained were of the same magnitude as those obtained with many primary antiknock materials at much higher concentrations, it is apparent that the aromatic chromium tricarbonyls are not acting in the manner of a primary antiknock agent. That is, the secondary additives are acting in conjunction with or co-acting with the tetraethyllead. As further confirmation of this, the following test was performed:

#### EXAMPLE II

Mesitylene chromium tricarbonyl was added in various concentrations to separate samples of the same olefin-isobutane alkylate which had been employed in the previous example, but which contained no primary antiknock agent. The Research octane numbers of these samples

were then compared with the previously determined octane numbers of the alkylate which contained no additives of any kind. The results were as follows:

Table II

|                                  | ANTIKNOCK ACTION OF AROMATIC CHROMIUM TRICARBONYL WITHOUT TETRAALKYLLEAD | OCTANE NUMBER        |
|----------------------------------|--------------------------------------------------------------------------|----------------------|
| Concentration (millimoles/gal.): |                                                                          | enhancement (Δ.O.N.) |
| 10                               | 5                                                                        | -0.3                 |
|                                  | 10                                                                       | -0.4                 |

Thus, it may be seen that the aromatic chromium tricarbonyls are in fact pro-knock agents in the absence of tetraalkyllead primary antiknock agents, which indicates clearly that their efficacy as antiknock agents arises from their cooperative action or co-action with the lead primary antiknock agents. Though analogous aromatic metal tricarbonyls can also be prepared from molybdenum and tungsten, these materials have been found to possess no antiknock activity either primary or secondary.

Referring once again to Table I, it will be observed that the effectiveness of the aromatic chromium tricarbonyls varies considerably with their concentration in the blend, and, concomitantly with the ratio of co-antiknock agent to tetraethyllead. These data indicate that the secondary antiknock agents are effective in concentrations as small as 0.5 millimole per gallon. The upper limit at which antiknock effects are obtained, however, varies considerably with the particular co-antiknock agent which is used. For example, while mesitylene and ortho xylene chromium tricarbonyls appear to be ineffective above about 6 or 7 millimoles per gallon (U.S.), toluene chromium tricarbonyl is effective at much higher concentrations, for example, up to about 15 millimoles per gallon. Even so, the maximum benefit obtainable in gasoline containing 3 cc. TEL per gallon will be obtained at co-antiknock concentrations of less than about 15 millimoles per gallon.

The concentration of the co-antiknock agent is more meaningful, however, when it is expressed in relation to the amount of primary antiknock agent which is used therewith. It has been found that the optimum concentration of the co-antiknock agents is the gasoline compositions of the invention is approximately proportional to the amount of primary antiknock agent also used in the gasoline. This phenomenon, of course, still further indicates the cooperative action of the co-antiknock agents with tetraalkyllead. The amount of co-antiknock agent relative to the primary antiknock agent is most conveniently expressed in terms of the "metal ratio" which is defined and used hereinafter to mean the weight ratio of metal (chromium) contained in the co-antiknock agent to metal (lead) contained in the tetraalkyllead primary antiknock agent. Thus, the aromatic chromium tricarbonyls are effective to raise the octane number of leaded gasoline when the metal ratio of the two antiknock additives is at least 0.01 gram of chromium contained in the co-antiknock agent present per gram of lead contained in the primary antiknock agent present. A minimum metal ratio of 0.015 is preferred.

The maximum metal ratio at which the co-antiknock additives may be employed to obtain significant co-antiknock benefits varies considerably among the various aromatic chromium tricarbonyls which have been found to be operable. However, in each case this maximum ratio will not exceed about 0.25 gm. Cr/gm. Pb. Moreover, it is preferred to that the metal ratio not exceed about 0.15. Thus the fuel compositions of the invention contain an octane number-improving amount of co-antiknock agent which corresponds to a metal ratio of at least 0.015 but not more than about 0.15 gram of chromium per gram of lead.

Though in the foregoing examples tetraethyllead was employed in concentrations of 3 cc./gal. (U.S.), it will be

recognized that the fuel compositions in accordance with the invention may contain any octane number-improving amount of tetraethyllead, e.g., as low as 0.5 cc. TEL/gal. to as high as 12 cc. TEL/gal., so long as the metal ratio is kept within the foregoing discussed limits.

From the preceding discussion and data, it is apparent that the aromatic chromium tricarbonyls are highly effective as co-antiknock agents in isoparaffinic and naphthenic hydrocarbons. However, their use as co-antiknock agents is not limited thereto. The composition of the base fuel to which they are added does, however, exert a profound effect on their activity as co-antiknock agent with tetraalkyllead compounds.

*Effect of iso and normal paraffins on co-antiknock activity.*—The addition of light isoparaffins, i.e., those having less than 8 carbon atoms per molecule, is beneficial to the action of the co-antiknock agent. However, the addition of heavier isoparaffins reduces the co-antiknock effect considerably. It is therefore preferred that the gasoline compositions in accordance with the invention not contain greater than about 20% by volume of isoparaffins boiling over about 300° F. It is even further preferred that the gasoline composition contain no more than about 10% by volume of isoparaffins boiling above about 300° F.

Because of the detrimental effect of normal paraffins in reducing the octane number, the gasoline compositions in accordance with the invention preferably contain essentially no normal paraffins having 7 or more atoms per molecule and only small amounts, preferably not over 10%, of normal paraffins having 5 or 6 carbon atoms per molecule. Fuel compositions containing essentially no normal paraffins having 5 or more carbon atoms per molecule are particularly preferred. Normal paraffins having less than 5 carbon atoms per molecule, for example, normal butane, having high octane numbers, are useful to provide the gasoline with proper vapor pressure and are not deleterious to the action of the co-antiknock agents.

*Effect of cycloparaffins (naphthenes).*—The gasoline compositions of the invention should contain no more than 10% by volume naphthenes boiling above about 300° F., and preferably substantially none, because they are deleterious both with regard to blending octane number and their effect on the response of the co-antiknock agent. There is no limit, however, in the broad aspects of the invention, to the maximum concentration of naphthenes 45 boiling below about 300° F.

*Effect of olefins on co-antiknock activity.*—The incorporation of up to about 10% of lighter olefins, especially those which are branched, is actually beneficial to the co-action of the co-antiknock agents with tetraethyllead. Moreover, the gasoline compositions of the invention can advantageously contain up to 30% by volume olefins, but larger quantities are deleterious and should be avoided.

*Effect of aromatics.*—Aromatics boiling below about 300° F., i.e., C<sub>8</sub> aromatic hydrocarbons and lighter, have been found to be not greatly deleterious in minor concentrations, e.g., below about 50% by volume. Heavier aromatics, however, which boil above about 300° F., are deleterious and should not exceed about 20% by volume of the total gasoline blend. In fact, in order to obtain more practical benefits from the co-antiknock agent, it is preferred that the gasoline of the invention contain no more than about 10% by volume of aromatics boiling above 300° F., and no more than 30% by volume of total aromatics.

Though the deleterious effect of high boiling aromatics on the effectiveness of the co-antiknock additives is quite unfortunate, it has been found that a very surprising relationship exists between the effect of heavy aromatics and the presence of light naphthenes. That is, light naphthenes suppress the deleterious effects of heavy aromatics. In accordance with applicants' copending patent application Serial No. 18,255, it is possible to have substantial amounts of aromatics boiling above 300° F. in a base gasoline and still obtain large benefits from co-antiknock

additives, as long as light naphthenes, i.e., naphthenes boiling below about 300° F., are also incorporated in the base gasoline.

Relatively high response is obtained in light naphthenes 5 even in the presence of heavy aromatics. In general it appears that one volume percent of light naphthenes can overcome completely the deleterious effect of one volume percent of heavy aromatics. However, since practical benefits are obtained up to 10% and 20% by volume 10 heavy aromatics even in the absence of naphthenes, it is not necessary always to have present as much light naphthenes as would be needed to completely cancel the effect of the heavy aromatics. The light naphthenes can be used to obtain even greater benefits from the co-antiknock additives in gasoline which must contain aromatics boiling above 300° F., to have proper volatility distribution of 15 high octane number components. To take advantage of light naphthenes in accordance with this preferred aspect of the invention, it is desirable that the base gasoline contain at least 1/4% by volume, or preferably at least 1/2% by volume, of naphthenes boiling below 300° F. for each 20 1% by volume of aromatics boiling above 300° F. in excess of 10% by volume of such aromatics, and preferably such amounts of light naphthenes for each 1% by 25 volume of all of such aromatics.

The adverse effect of each of the deleterious or antagonistic components, that is, aromatics, olefins, C<sub>5</sub> plus normal paraffins and heavy naphthenes, is not, however, independent. Even with the use of naphthenes in accordance 30 with above, the presence of two or more of such antagonists in maximum concentrations can result in a fuel having little or no response to the action of the co-antiknock agents. Such non-responsive hydrocarbon compositions may be avoided, however, if the compositions meet the 35 following empirical correlation which constitutes a limitation on the total equivalent amount of co-antiknock antagonists (A<sub>E</sub>) which may be present in the hydrocarbon blend:

$$A_E = A_L + 1.3A_H + 0.7A_O + 0.25A_P \leq 50 + 0.75N$$

wherein

A<sub>L</sub>=percent by volume of aromatics boiling below 300° F.

A<sub>H</sub>=percent by volume of aromatics boiling above 300° F.

A<sub>O</sub>=percent by volume of olefins

A<sub>P</sub>=percent by volume of C<sub>5</sub> plus normal paraffins and naphthenes boiling above 300° F.

N=percent by volume of naphthenes boiling below 300° F.

Summing up its broad aspects, the invention therefore resides in the discovery that aromatic chromium tricarbonyls, as defined hereinbefore, are effective as co-antiknock agents with tetraethyllead when both are added to gasoline blends containing essentially no normal paraffins 55 containing 7 or more carbon atoms, no more than 10% by volume of C<sub>5</sub> to C<sub>6</sub> normal paraffins, no more than 20% by volume of isoparaffins boiling above 300° F., no more than 10% by volume of naphthenes boiling above 300° F., no more than 30% by volume olefins, no more than 50% by volume of total aromatics and no more than 20% by volume of aromatics boiling above 300° F., the composition of the gasoline blend also being within the limits defined by the empirical relationship

$$A_E = A_L + 1.3A_H + 0.7A_O + 0.25A_P \leq 50 + 0.75N$$

In the foregoing examples in which TEL was used as primary anti-detonant, the TEL was added in the form of the commercial motor mix which has the following composition.

| Component:              | Percent by weight |
|-------------------------|-------------------|
| Tetraethyllead          | 61.48             |
| Ethylene dibromide      | 17.86             |
| Ethylene dichloride     | 18.81             |
| Dye                     | 0.06              |
| Kerosene and impurities | 1.79              |

The co-antiknock materials of the invention are, however, equally effective in leaded gasoline in which pure TEL, and no halohydrocarbon scavenger, is used, or in which the commercial aviation mix containing one theory of ethylene dibromide, and no ethylene chloride, is used.

Besides the aforementioned halogen-containing lead scavengers, the fuel compositions of the invention can, and ordinarily will, contain other additives, for example, dyes, spark plug anti-foulants such as tricresyl phosphate, dimethyl xylyl phosphate, and diphenyl cresyl phosphate, combustion modifiers such as alkyl boronic acids and lower alkyl phosphates and phosphites, oxidation inhibitors such as N,N'-disalicylal-1,2-propanediamine, and rust inhibitors such as polymerized linoleic acids and N,C-disubstituted imidazolines, and the like.

It is to be understood that the order of mixing the various constituents of the compositions of the invention is immaterial. For example, the co-antiknock compound may be added to a gasoline which already contains the tetraalkyllead primary antiknock material. Likewise, the co-antiknock and primary antiknock compounds may be first mixed, stored, and handled as a concentrate, and added to the gasoline at a later time. A gasoline additive concentrate of this latter type may also contain halogen scavenger and spark plug antifouling compound. Under other circumstances, it may be desirable to mix the halogen scavenger and the primary antiknock compound, or the primary antiknock and co-antiknock compounds, in the desired relative proportions and handle or store this mixture, with or without stabilizers, antifouling compounds, inhibitors, etc., as a concentrate for incorporation with the other components of the ultimate fuel composition.

An additive concentrate of this latter type will therefore contain from 0.01 to 0.25 gram of metal in the co-antiknock agent per gram of lead in the tetraalkyllead. Preferably, such a concentrate contains from about 0.015 to about 0.15 gram of metal per gram of lead. A typical additive concentrate in accordance with the invention and containing both TEL motor mix and phosphorus compound for ignition control as well as co-antiknock agent has the following composition.

| Component:                                 | Percent by weight |
|--------------------------------------------|-------------------|
| Tetraethyllead                             | 49.0-58.9         |
| Ethylene dibromide                         | 14.2-17.1         |
| Ethylene dichloride                        | 15.0-18.1         |
| Phosphorus (as tricresyl phosphate)        | 3.8-12.5          |
| Chromium (as toluene chromium tricarbonyl) | 0.4-7.9           |
| Kerosene, dye, impurities                  | 1.4-1.7           |

We claim as our invention:

1. A gasoline composition consisting essentially of a mixture of hydrocarbons having an ASTM boiling range below about 400° F., an octane number-improving amount of tetraalkyllead and an octane number-improving amount of an aromatic chromium tricarbonyl co-antiknock agent corresponding to the formula  $ACr(CO)_3$ , wherein A is a monoaromatic compound corresponding to the formula



wherein the R groups are monovalent radicals, three of which are selected from the group consisting of —H and —CH<sub>3</sub>, and one of which is selected from the group consisting of —H and —C<sub>n</sub>H<sub>2n+1</sub>, wherein n is a whole number of from 1 to 4 inclusive, and the R' groups are selected from the group consisting of —H and —CH<sub>3</sub> when separate and (—CH<sub>2</sub>)<sub>4</sub> when taken together, the amount of said co-antiknock agent corresponding to from about 0.01 to about 0.25 gram of chromium contained in the co-antiknock agent per gram of lead contained in the tetraalkyllead, said mixture of hydrocarbons contain-

ing (1) no more than 50% by volume of aromatics, (2) no more than about 30% by volume olefins, (3) no more than about 20% by volume each of isoparaffins and aromatics boiling above about 300° F., (4) no more than about 10% by volume each of normal paraffins having 5 to 6 carbon atoms per molecule and naphthenes boiling above about 300° F., and (5) essentially no normal paraffins having greater than 6 carbon atoms per molecule, and further characterized as having an equivalent amount of co-antiknock antagonists (A<sub>E</sub>) not exceeding 50+0.75N wherein A<sub>E</sub> and N are defined as hereinbefore in the specification.

2. The fuel composition of claim 1 containing (1) no more than 50% by volume of aromatics, (2) no more than about 20% by volume each of olefins and aromatics boiling above about 300° F., (3) no more than about 10% by volume each of isoparaffins boiling above about 300° F. and naphthenes boiling above about 300° F., and (4) essentially no normal paraffins having greater than 4 carbon atoms per molecule, and further characterized as having an equivalent amount of co-antiknock antagonists (A<sub>E</sub>) not exceeding 50+0.75N wherein A<sub>E</sub> and N are defined as hereinbefore in the specification.

3. A gasoline composition consisting essentially of a mixture of hydrocarbons having an ASTM boiling range below about 400° F., an octane number-improving amount of tetraalkyllead and an octane number-improving amount of mesitylene chromium tricarbonyl co-antiknock agent corresponding to from about 0.01 to about 0.25 gram of chromium contained in the co-antiknock agent per gram of lead contained in the tetraalkyllead, said mixture of hydrocarbons containing (1) no more than 50% by volume of aromatics, (2) no more than about 30% by volume olefins, (3) no more than about 20% by volume each of isoparaffins and aromatics boiling above about 300° F., (4) no more than about 10% by volume each of normal paraffins having 5 to 6 carbon atoms per molecule and naphthenes boiling above about 300° F., and (5) essentially no normal paraffins having greater than 6 carbon atoms per molecule, and further characterized as having an equivalent amount of co-antiknock antagonists (A<sub>E</sub>) not exceeding 50+0.75N wherein A<sub>E</sub> and N are defined as hereinbefore in the specification.

4. A gasoline composition consisting essentially of a mixture of hydrocarbons having an ASTM boiling range below about 400° F., an octane number-improving amount of tetraalkyllead and an octane number-improving amount of toluene chromium tricarbonyl co-antiknock agent corresponding to from about 0.01 to about 0.25 gram of chromium contained in the co-antiknock agent per gram of lead contained in the tetraalkyllead, said mixture of hydrocarbons containing (1) no more than 50% by volume of aromatics, (2) no more than about 30% by volume olefins, (3) no more than about 20% by volume each of isoparaffins and aromatics boiling above about 300° F., (4) no more than about 10% by volume each of normal paraffins having 5 to 6 carbon atoms per molecule and naphthenes boiling above about 300° F., and (5) essentially no normal paraffins having greater than 6 carbon atoms per molecule, and further characterized as having an equivalent amount of co-antiknock antagonists (A<sub>E</sub>) not exceeding 50+0.75N wherein A<sub>E</sub> and N are defined as hereinbefore in the specification.

5. A gasoline composition consisting essentially of a mixture of hydrocarbons having an ASTM boiling range below about 400° F., an octane number-improving amount of tetraalkyllead and an octane number-improving amount of ortho xylene chromium tricarbonyl co-antiknock agent corresponding to from about 0.01 to about 0.25 gram of chromium contained in the co-antiknock agent per gram of lead contained in the tetraalkyllead, said mixture of hydrocarbons containing (1) no more than 50% by volume of aromatics, (2) no more than about 30% by volume olefins, (3) no more than about 20% by volume each of isoparaffins and aromatics boiling above about 300° F., (4) no more than about 10% by volume each of normal paraffins having 5 to 6 carbon atoms per molecule and naphthenes boiling above about 300° F., and (5) essentially no normal paraffins having greater than 6 carbon atoms per molecule, and further characterized as having an equivalent amount of co-antiknock antagonists (A<sub>E</sub>) not exceeding 50+0.75N wherein A<sub>E</sub> and N are defined as hereinbefore in the specification.

mal paraffins having 5 to 6 carbon atoms per molecule and naphthenes boiling above about 300° F., and (5) essentially no normal paraffins having greater than 6 carbon atoms per molecule, and further characterized as having an equivalent amount of co-antiknock antagonists ( $A_E$ ) not exceeding  $50+0.75N$  wherein  $A_E$  and  $N$  are defined as hereinbefore in the specification.

6. A gasoline additive concentrate composition consisting essentially of a mixture of tetraalkyllead and an aromatic chromium tricarbonyl co-antiknock agent, the amount of co-antiknock agent corresponding to the formula  $ACr(CO)_3$ , wherein  $A$  is a monoaromatic compound corresponding to the formula



wherein the  $R$  groups are monovalent radicals, three of which are selected from the group consisting of  $-H$  and  $-CH_3$ , and one of which is selected from the group consisting of  $-H$  and  $-CnH_{2n+1}$ , wherein  $n$  is a whole number of from 1 to 4 inclusive, and the  $R'$  groups are selected from the group consisting of  $-H$  and  $-CH_3$  when separate and  $(-CH_2-)_4$  when taken together, corre-

sponding to from about 0.01 to about 0.25 gram of chromium contained in the co-antiknock agent per gram of lead contained in the tetraalkyllead.

5      References Cited in the file of this patent  
UNITED STATES PATENTS

|    |           |                       |                |
|----|-----------|-----------------------|----------------|
| 10 | 2,086,775 | Lyons et al. -----    | July 13, 1937  |
|    | 2,197,498 | Guthmann -----        | Apr. 16, 1940  |
|    | 2,460,700 | Lyons -----           | Feb. 1, 1949   |
|    | 2,818,416 | Brown et al. -----    | Dec. 31, 1957  |
|    | 2,875,223 | Pedersen et al. ----- | Feb. 24, 1958  |
|    | 2,913,413 | Brown -----           | Nov. 17, 1959  |
|    | 3,001,858 | Antonsen -----        | Sept. 26, 1961 |

15      OTHER REFERENCES

- “A General Method of Preparing Tricarbonylchromium Derivatives of Aromatic Compounds,” by Nicholls et al., Proceedings of the Chemical Society, London, May 20 1958, pp. 152 and 153.
- “Improved Motor Fuels Through Selective Blending,” by Wagner et al., Paper presented before 22nd Annual Meeting of the American Petroleum Institute, November 7, 1941, pp. 70-89.
- 25      “Aviation Gasoline Manufacture,” by Van Winkle, First Ed., 1944, McGraw-Hill Book Co., pp. 43-63 and 197-211.